# EUROPEAN PATENT SPECIFICATION

(11) **EP 3 151 988 B1**
(45) Date of publication and mention of the grant of the patent: **17.01.2018**
(21) Application number: 14736027.5
(22) Date of filing: 09.06.2014
(51) Int. Cl.: B21D 51/26, C22C 29/08, C22C 29/02

(54) **CEMENTED CARBIDE NECKING TOOL**
AUSHALSMEISSEL FÜR ZEMENTIERTES CARBID
OUTIL DE STRICTION DE CARBURE CÉMENTÉ

(43) Date of publication of application: 12.04.2017
(73) Proprietor: Sandvik Intellectual Property AB, 811 81 Sandviken (SE)
(72) Inventor: HEWITT, Stephen, A., Coventry West Midlands CV4 9TH (GB); TARRES PUIT, Elena, Coventry West Midlands CV5 7AN (GB); RIMBAU, Victor, 08015 Barcelona (ES)
(74) Representative: Neilson, Martin Mark
(86) International application number: PCT/IB2014/062073
(87) International publication number: WO 2015/189654

(56) References cited:
- EP-A1- 2 439 294
- EP-A1- 2 460 598
- WO-A1-01/14608
- WO-A1-2008/147487
- WO-A1-2009/094763
- US-A- 5 736 658
- US-A1- 2012 312 066

## Description

### TECHNICAL FIELD AND INDUSTRIAL APPLICABILITY

The present invention relates to a cemented carbide necking tool having lower density, higher hardness, and closer thermal expansion to tool steel for applications in the can manufacturing industry.

### BACKGROUND

Over 280 billion beverage cans are produced worldwide every year. During the process, the upper section of the can is reduced in a necking-in operation to accommodate a top. Dies are commonly used in the necking operation. Due to the large number of cans produced service life of the die tool is crucial.

Accordingly, the necking die material must satisfy the most demanding applications. Cemented carbide, which is produced using modern powder metallurgical processes, offers a unique combination of strength, hardness and toughness. Cemented carbide, as used herein, is defined as a hard, carbide phase, 70 to 97 wt-% of the composite and a binder phase. Cemented carbides include standard WCCo, Cermets and hybrids. Tungsten carbide (WC) is the most common hard phase and cobalt (Co) the most common binder phase. These two materials form the basic cemented carbide structure. From this basic concept many other types of cemented carbide have been developed. In addition to WC-Co compositions, varying proportions of titanium carbide (TiC), tantalum carbide (TaC) or niobium carbide (NbC) or others can be used. In addition, the cobalt binder phase can be alloyed with or completely replaced by nickel (Ni), chromium (Cr), iron (Fe), molybdenum (Mo) or alloys of these elements.

By varying the composition, the resulting physical and chemical properties can be tailored to ensure maximum resistance to wear, deformation, fracture, corrosion, oxidation and other damaging effects. The available unique composition of cemented carbide makes it an ideal tool material for forming and stamping in the can making process. An example of a known die 10 is illustrated in Fig. 1. Typical necking dies work with knock out that is normally made of tool steel due to reduced cost. The match gap of the knock out and necking dies must be kept as constant as possible during start up and running conditions of the necker machine, therefore the closer the thermal expansion of the necking die to the tool steel the better.

EP2439294, assigned to the assignee of the present invention, discloses a cemented carbide punch used for the manufacturing of metal beverage cans. The particular disclosed cemented carbide has a hard phase of WC and a binder phase based on Co and Ni. The composition comprises, in wt-%, from 50 to 70 WC, from 15 to 30 TiC (titanium carbide) and from 12 to 20 Co +Ni. The punch application is particularly suited to this particular composition as the weight of the punch can be lowered and production speeds increased.

WO2008079083, also assigned to the assignee of the present invention, discloses a cemented carbide punch used in cold forming and drawing operations, particularly in the manufacture of beverage cans. The cemented carbide is essentially, in wt %: 70-90 WC; 2-8 TiC, 1-9 NbC, 0-3 TaC and 5-20 binder phase of Co with an addition of Cr and possibly one or more of the elements selected from Ni, Fe and Mo. More particularly the binder composition is, also in wt %: 10-98 Co, 0-50 Ni, 2-15 Cr, 0-50 Fe and 0-10 Mo.

Further, grades with binder content in the range of 3 to 10 wt % and grain sizes below 1 µm have the highest hardness and compressive strength, combined with high wear resistance and high reliability against breakage. As used herein grade can be defined as tungsten carbide (WC) in combination with a binder phase of cobalt (Co) and/or nickel (Ni), and any other single or combination of carbide phases (TiC, Ta/NbC etc.). However, the binder phase of cemented carbides is susceptible to wet corrosion resulting in wear problems. Accordingly, sub-micron carbide grains combined with the appropriate binder have been used in WC-Co carbide punches.

However, such materials have not been previously used for necking dies.

### SUMMARY

In one aspect there is provided a necking tool for manufacturing of metal beverage cans, the necking tool being a cemented carbide containing in wt % of 18 - 63WC; 21 - 30 TiC; 0 - 27 TiN; 0 - 12 NbC; 0 - 2 Cr₃C₂; 8 - 14 Co and 0 - 6 Ni.

According to another aspect there is provided a necking tool for manufacturing of metal beverage cans, the necking tool being a cemented carbide including in wt % of less than 63 WC; 21 TiC; 2 Cr3C2; 8 Co; and less than 6 Ni.

In yet another aspect there is provided a necking tool for manufacturing of metal beverage cans, the necking tool being a cemented carbide including in wt % of 18 WC; less than 30 TiC; less than 27 TiN; less than 12 NbC, and 14 Co.

These and other objects, features, aspects, and advantages of the present invention will become more apparent from the following detailed description of the preferred embodiment relative to the accompanied drawings, in which:

### BRIEF DESCRIPTION OF THE DRAWINGS

Fig. 1 is a perspective view of a known necking die used in manufacturing metal beverage cans.
Fig. 2 is a SEM image of a first necking tool material according to the present disclosure.
Fig. 3 is a SEM image of a second necking tool material according to the present disclosure.
Fig. 4 is a SEM image of the porosity level of Sample B of Fig. 3.

### DETAILED DESCRIPTION

The present invention relates to cemented carbide including hybrids and cermets for necking applications in the can manufacturing industry. The advantages associated with these new materials can be seen in higher hardness, lower density, and closer thermal expansion to a tool steel knock-out and enhanced toughness compared to existing ceramic material used for necking dies

Cemented carbide grades with the compositions in wt % according to Table 1 below were produced according to known methods. The cemented carbide samples were prepared from powders forming the hard constituents and powders forming the binder, which were wet milled together, dried, pressed into bodies of desired shape and sintered.

**Table 1**

| GRADE | WC | TiC | TiN | NbC | Cr₃C₂ | Co | Ni |
|---|---|---|---|---|---|---|---|
| SAMPLE A | 63.00 | 21.00 | 0.00 | 0.00 | 2.00 | 8.00 | 6.00 |
| SAMPLE B | 18.00 | 30.00 | 27.00 | 12.00 | 0.00 | 14.00 | 0.00 |
| COMPARATIVE | 88.0 | 0.00 | 0.00 | 0.00 | 1 | 12 | 0.00 |

A known cemented carbide, Sandvik grade H12N, (Sandvik AB, Sandviken, SE), used in the can tooling industry, was used as the comparative sample. The comparative sample contains in wt% less than about 88 WC; about 12 Co; and about 1 Cr₃C₂, preferably 87.5% WC, 12%Co and 0.5 Cr₃C₂. Moreover, the comparative sample has a medium carbide grain size, a corrosion resistance on a subjective scale of 1 to 10 of about 3, a wear resistance on a subjective scale of 1 to 10 of about 5, a compressive strength of about 4600 MPa, and a fracture toughness, per the Palmqvist method, of about 16 MPa m^{1/2}.

### Example

Two cemented carbide bodies according to the present disclosure were prepared and characterized (Samples A and B) as shown in Table 1. The samples were analyzed by electron microscopy. The SEM micrograph of Sample A is shown in Fig. 2 and Sample B is shown in Fig. 3. As shown, it can be seen that the morphology and distribution of the hard and matrix phases are uniform.

Both Sample A and B have a grain size from 0.5 µm to 1 µm. The binder content for both samples is approximately 14%. Preferably, 6 to 18% Co/Ni.

According to one aspect, the necking tool is made of a cemented carbide including in wt % of 18 - 63 WC; less than 30 TiC; 0 - 27 TiN; 0 - 12 NbC; 0 - 2 Cr₃C₂; 8 - 14 Co; and 0 - 6 Ni.

According to another aspect, the necking tool is made of cemented carbide including in wt % less than 63 WC, and more preferably 62.8 WC; 21 TiC; 2 Cr3C2; 8 Co and more preferably 8.3 Co; and less than 6 Ni and more preferably 5.7 Ni. Accordingly, the binder phase consists of Co and Ni and has a content of approximately 14 wt %.

In another aspect, the necking tool is made of a cemented carbide including in wt-%, of 18 WC, and more preferably, 18.08 WC; less than 30 TiC, and more preferably 29.66 TiC; less than 27 TiN, and more preferably 26.46 TiN; less than 12 NbC, and more preferably 11.63; and 14 Co and more preferably 14.17 Co.

Referring to Table 1 and as can be seen in Fig. 3, Sample B utilizes N to inhibit grain growth. Moreover, the Ti grains are spherical and the Co binder well distributed. Also, as shown in Fig. 4, the optical micrograph shows A02/A04 type porosity levels.

Other properties were measured according to standards used in the cemented carbide industry as shown in Table 2 below.

**Table 2**

| | Density (g/cm³) | Hardness (kg/mm²) | Young's Modulus (GPa) | Coefficient of thermal expansion 20-200°C (1x10⁻⁶/°C) |
|---|---|---|---|---|
| Sample A | 9.86 | 1450 | 440 | 7.13 |
| Sample B | 6.62 | 1650 | 400 | 7.49 |
| Comparative | 14.25 | 1335 | 590 | 5.41 |

As can be seen, Samples A and B have a much higher hardness, of 1450 and 1650 respectively and a much lower density, of less than 10 g/cm³, than the comparative H12N, of 9.86 and of 6.62 respectively, and closer thermal expansion, of 7.13 and of 7.49, to known tool steel.

Although the present invention has been described in relation to particular embodiments thereof, many other variations and modifications and other uses will become apparent to those skilled in the art. It is preferred therefore, that the present invention be limited not by the specific disclosure herein, but only by the appended claims.

## Claims

1. A necking tool for manufacturing of metal beverage cans, the necking tool being a cemented carbide comprising in wt % of 18 - 63 WC; 21- 30 TiC, 0- 27 TiN; 0-12 NbC; 0 to 2 Cr₃C₂; 8 to 14 Co; and 0 to 6 Ni.

2. A necking tool according claim 1, wherein a binder content of the cemented carbide is about 14 wt %.

3. A necking tool according to any one of the preceding claims, wherein the cemented carbide has a density of less than 10 g/cm³.

4. A necking tool according to any one of the preceding claims, wherein the cemented carbide has a coefficient of thermal expansion of 7.13 1x10⁻⁶/°C.

5. A necking tool according to any of the preceding claims, wherein a binder content of the cemented carbide is 14.17 wt %.

6. A necking tool according to any of the preceding claims, wherein the cemented carbide has a coefficient of thermal expansion of 7.49 1x10⁻⁶/°C

7. A necking tool according to any one of the preceding claims, wherein the cemented carbide has a grade with a grain size less than 1 µm, preferably 0.5 to 1 µm, and more preferably 0.5 to 0.9 µm.

8. Use of a necking tool according to any of the preceding claims for manufacturing a metal beverage can.

## Patentansprüche

1. Aushalswerkzeug zur Herstellung von Metallgetränkedosen, wobei das Aushalswerkzeug ein zementiertes Carbid ist, umfassend in Gew.-% 18-63 WC; 21-30 TiC; 0-27 TiN; 0-12 NbC; 0 bis 2 Cr₃C₂; 8 bis 14 Co und 0 bis 6 Ni.

2. Aushalswerkzeug gemäß Anspruch 1, wobei ein Bindemittelgehalt des zementierten Carbids etwa 14 Gew.-% ist.

3. Aushalswerkzeug gemäß einem der vorangehenden Ansprüche, wobei das zementierte Carbid eine Dichte von weniger als 10 g/cm³ hat.

4. Aushalswerkzeug gemäß einem der vorangehenden Ansprüche, wobei das zementierte Carbid einen Wärmeausdehnungskoeffizienten von 7,13 1x10⁻⁶/°C hat.

5. Aushalswerkzeug gemäß einem der vorangehenden Ansprüche, wobei der Bindemittelgehalt des zementierten Carbids 14,17 Gew.-% ist.

6. Aushalswerkzeug gemäß einem der vorangehenden Ansprüche, wobei das zementierte Carbid einen Wärmeausdehnungskoeffizienten von 7,49 1x10⁻⁶/°C hat.

7. Aushalswerkzeug gemäß einem der vorangehenden Ansprüche, wobei das zementierte Carbid eine Qualität mit einer Korngröße von weniger als 1 µm, vorzugsweise von 0,5 bis 1 µm und bevorzugter von 0,5 bis 0,9 µm hat.

8. Verwendung eines Aushalswerkzeugs gemäß einem der vorangehenden Ansprüche zur Herstellung einer Metallgetränkedose.

## Revendications

1. Outil à rétreindre destiné à fabriquer des canettes de boisson en métal, l'outil à rétreindre étant un carbure cémenté comprenant en % en poids 18 à 63 WC ; 21 à 30 TiC, 0 à 27 TiN ; 0 à 12 NbC ; 0 à 2 Cr₃C₂ ; 8 à 14 Co ; et 0 à 6 Ni.

2. Outil à rétreindre selon la revendication 1, dans lequel une teneur en liant du carbure cémenté est d'environ 14 % en poids.

3. Outil à rétreindre selon l'une quelconque des revendications précédentes, dans lequel le carbure cémenté a une masse volumique de moins de 10 g/cm³.

4. Outil à rétreindre selon l'une quelconque des revendications précédentes, dans lequel le carbure cémenté a un coefficient de dilatation thermique de 7,13 1 x 10⁻⁶/°C.

5. Outil à rétreindre selon l'une quelconque des revendications précédentes, dans lequel une teneur en liant du carbure cémenté est de 14,17 % en poids.

6. Outil à rétreindre selon l'une quelconque des revendications précédentes, dans lequel le carbure cémenté a un coefficient de dilatation thermique de 7,49 1 x 10⁻⁶/°C.

7. Outil à rétreindre selon l'une quelconque des revendications précédentes, dans lequel le carbure cémenté a une grosseur de grain de moins de 1 µm, de préférence de 0,5 à 1 µm, et de manière davantage préférée de 0,5 à 0,9 µm.

8. Utilisation d'un outil à rétreindre selon l'une quelconque des revendications précédentes, pour fabriquer une canette de boisson en métal.
